

Patented May 29, 1923.

1,457,288

# UNITED STATES PATENT OFFICE.

PETER OSTENDORF, OF BERNDORF, AUSTRIA.

## BRONZE ALLOY AND PROCESS FOR ITS PRODUCTION.

No Drawing.

Application filed October 4, 1922. Serial No. 592,410.

To all whom it may concern:

Be it known that I, PETER OSTENDORF, a Prussian subject, residing at Berndorf, Lower Austria, have invented new and useful Improvements in and Relating to Bronze Alloys and Processes for Their Production, of which the following is a specification.

The present invention relates to novel bronze alloys which in their composition 10 closely resemble genuine bronzes, but differ from them essentially and advantageously, in that they are capable of being easily worked in the cold state and also possess whilst in the hot state, an adequate degree 15 of suitability for working.

It is well known, that genuine bronzes, consisting of copper and tin, are in practice almost unworkable, and therefore have a very limited range of use. In particular, 20 such bronzes cannot be employed for the manufacture of such parts as require, after the casting operation, a further tooling of any kind. On the other hand it would be desirable, for many purposes, if the good 25 properties of these genuine bronzes could be utilized.

Attempts have, in fact, already been made at improving bronzes consisting of copper and tin by the addition of other metals such 30 as nickel and zinc. In such alloys, however, the percentage of tin was comparatively small, whilst the percentage of zinc was comparatively large, and, therefore, products resulted which were not serviceable for practical purposes, and which did not show, in an 35 adequate measure, the desirable properties of genuine bronzes.

The invention consists in compounding 87 parts by weight of copper with 4.5-10 parts 40 by weight of tin, 1-5 parts by weight of nickel and not more than 5 parts by weight of zinc to produce the improved bronze alloy.

According to this invention, important 45 improvements of copper and tin alloys are obtained by making suitable additions of nickel and zinc and by suitably adjusting the proportions of these additions it is possible to produce, a softer or harder material 50 as required. Bronzes made in accordance with this invention consist, generally speaking, of at least 87 parts of copper, 4.5-10 parts of tin, 1-5 parts of nickel and not more than 5 parts of zinc. In compounding the 55 alloy, the copper and nickel are first melted together, then the tin is added, and finally

the zinc. A percentage of zinc exceeding 5% is not admissible, because zinc has the property of rendering the alloy soft but this softening is only obtained when the percentage of zinc does not exceed 5%, if the percentage of zinc is increased beyond this limit, the alloy again becomes harder.

Castings suitable for use with superheated steam can be produced if the improved 65 alloys, as such alloys can be relied upon to stand temperatures up to 500° (C.), which is due to the fact that the cast metal is very dense and articles made therefrom are not liable to be influenced by high pressure at 70 high temperatures.

By suitable variation in the proportion of the constituents of the alloy softer or harder bronzes can be produced. For example:—a soft bronze, which is particularly well suited 75 for wires for paper manufacture, and for other fine wires, may be composed of 87 parts of copper, 7 parts of tin, 1-5 parts of nickel, and 4.5 parts of zinc. Such an alloy, when drawn into wire, and annealed so as to be 80 softened, has a tensile strength of 28½ tons per square inch with 60-65% elongation whilst hard-drawn wires of the alloy have a tensile strength of up to 66½ tons per square 85 inch.

A harder alloy which is particularly suited for the manufacture of springs of all kinds, for example:—the springs of press buttons, in which it is of importance to have an exceedingly strong material which will 90 retain its resilience:—contact blades for telephonic and similar apparatus and many other like purposes, with great advantage, may consist of 88 parts of copper, 7.5 parts of tin, 2.5 parts of nickel and 2 parts of zinc. 95 This material, when drawn and annealed so as to be softened has a tensile strength of 35 tons per square inch with about 45% elongation.

The new bronze alloys composed in accordance with this invention are much superior, for many purposes of use, to any of the materials now available, and it has already been ascertained by experiments, that paper-making wires of a soft bronze alloy 100 as hereinabove described are still perfectly serviceable after a period of use twice as long as that obtainable with the best paper-making wires hitherto available.

I claim:

1. An improved bronze alloy consisting of not less than 87 parts by weight of cop-

per,  $4\frac{1}{2}$  to 10 parts by weight of tin, 1 to 5 parts by weight of nickel and 1 to 5 parts by weight of zinc.

2. An improved bronze alloy consisting of 5 88 parts by weight of copper,  $7\frac{1}{2}$  parts by weight of tin,  $2\frac{1}{2}$  parts by weight of nickel and 2 parts by weight of zinc.

3. A process for obtaining an improved bronze alloy consisting in melting the copper together with the nickel, adding the tin

to the molten mixture and finally adding the zinc.

In testimony whereof I have signed this specification in the presence of two witnesses.

P. OSTENDORF.

Witnesses:

CARL WIEDENBERG,  
JOHANN KUHN.